# EUROPEAN PATENT SPECIFICATION

(11) **EP 0 539 417 B1**
(45) Date of publication and mention of the grant of the patent: **19.06.1996**
(21) Application number: 91912577.3
(22) Date of filing: 12.07.1991
(51) Int. Cl.: C22C 1/10, B22D 27/20

(54) **CAST COMPOSITE MATERIALS**
GEGOSSENES VERBUNDMATERIAL
MATERIAUX COMPOSITES COULES

(30) Priority: 16.08.1990 US 572218; 26.07.1990 US 558630
(43) Date of publication of application: 05.05.1993
(62) Divisional of application: 95108612.3
(73) Proprietor: ALCAN INTERNATIONAL LIMITED, Montreal Quebec H3A 3G2 (CA)
(72) Inventor: SKIBO, Michael, D., Leucadia, CA 92024 (US); HAMMOND, Donald, E., San Diego, CA 92127 (US)
(74) Representative: Gaunt, Robert John
(86) International application number: CA9100242
(87) International publication number: WO9201821

(56) References cited:
- DE-C- 3 807 541

## Description

### TECHNICAL FIELD

This invention relates to the preparation of cast composite materials having matrix alloys that do not readily wet the reinforcement particles, and to cast metal-matrix composite materials, particularly composites having a matrix alloy tailored to avoid the formation of harmful intermetallic phases.

### BACKGROUND ART

Cast composite materials are conventionally formed by melting a matrix alloy in a reactor and then adding particles. The mixture is vigorously mixed to encourage wetting of the matrix alloy to the particles, and after a suitable mixing time the mixture is cast into molds or forms. The mixing is conducted while minimizing the introduction of gas into the mixture. The cast composite materials have fully wetted particles, few voids, and a generally uniformly mixed structure. Complete wetting is necessary to realize the full composite strength and other mechanical properties.

Such cast composite materials are much less expensive to prepare than other types of metal-matrix composite materials such as those produced by powder metallurgical technology. Composite materials produced by this approach, as described in US Patents 4,759,995 and 4,786,467, have enjoyed commercial success in only a few years after theirs first introduction.

As the cast composite materials have entered commercial production, customers have sometimes requested particle/matrix alloy combinations wherein the matrix does not readily wet the particles. In other instances, new metallic alloys have been identified that produce unexpectedly superior performance when used as the matrix phase of the composite materials, except for the problem that the composite materials are difficult to produce commercially due to the inability of the matrix alloy to wet and mix with the particles readily.

There are a number of techniques that can be applied to enhance wetting, which may work in some circumstances. The particles can be modified with special coatings, but the coating operation can significantly raise the cost of the particles and the composite material. Small amounts of reactive gases can be introduced into the mixing chamber, but the improved wetting may only be achieved at the cost of increased porosity in the cast composite material. Special reactive alloying ingredients can be added to the melt, but these are often expensive and may have adverse consequences in the production of undesired minor phases in the cast composite material. Another approach is to raise the temperature at which the mixing to achieve wetting is accomplished, but increased temperature may also result in the acceleration of the production of deleterious minor phases where such phases are thermodynamically favored but kinetically slow in forming at lower temperatures.

There therefore exists a continuing need for an improved technique for producing cast composite materials from particle/matrix alloy combinations wherein the matrix does not inherently readily wet the particle. Desirably, any such technique would not add substantially to the cost of the product or have detrimental effects.

One potential application of cast composite materials is in foundry remelt alloys. The composite materials are prepared by a supplier and cast into ingots at the supplier's plant. The cast ingots are transported to a commercial foundry, where they are remelted and cast to the final shape required by the customer. This foundry remelt approach is commonplace throughout industry for the processing of conventional aluminum alloys, and the introduction of aluminum-based cast composite materials into many applications is practical only where they can conform to this approach.

Experience has shown that, with the proper mixing technique, a wide variety of cast composite materials can be mixed by the suppliers. In the mixing step, the maximum temperature to which the molten composite may be heated is normally limited to avoid the production of unwanted reaction products between the matrix alloying elements and the reinforcement particles. Some reaction products can reduce the mechanical properties of the composite material and cause porosity in the composite material, and are therefore to be avoided.

However, many of these cast composite materials are not compatible with commercial foundry remelt practices. Cast composite materials used in remelt applications must permit high remelt temperatures, typically greater than those used in the composite mixing operation, and long remelt holding times. The casting of metallic composite materials into complex shapes requires that the molten material can be superheated above its melting point and be highly fluid so that it can flow into cold mold cavities for a considerable distance before the superheat is removed and the metal freezes. The greater is the remelt temperature permitted for the material and the fluidity of the material, the greater is the distance the molten composite material may flow into mold cavities before it solidifies, and the more intricate the products that can be cast.

Additionally, present foundry techniques usually call for the melting of large masses of the casting alloy to reach a stable temperature distribution, and casting articles from the large melted mass. The remelted material may remain at elevated temperature for extended periods of time, such as up to 24 hours, before casting. During this holding period, the castability of the composite material may degrade, so that a composite material may be much less castable after such a holding period than if cast immediately upon remelting. It is important that the composite material be castable by such commercial practices that have been long established, to accelerate the acceptance of the composite material by foundrymen.

In one specific example, aluminum-7 weight percent silicon alloys have been used in industry for years as remelt alloys, because the alloy has good fluidity and acceptable mechanical properties after casting. A satisfactory composite material of, for example, 15 volume percent of silicon carbide particles in an aluminum-7 weight percent silicon alloy may be prepared and cast by the supplier with a maximum temperature of 685°C in the mixing process. Ingots of this alloy are furnished to a foundry remelter, who remelts the ingots and holds the molten composite at a conventional remelt temperature of about 788°C for 8 hours before casting. The molten composite material casts very poorly, has low fluidity, and results in unacceptable product. The composite material is therefore rejected for the particular application, even though it might otherwise provide important benefits to the final product.

There therefore exists a need for an improved approach to the preparation of cast composite materials, particularly those for use in foundry remelt applications. The present invention fulfills this need, and further provides related advantages.

### DISCLOSURE OF INVENTION

One feature of the present invention provides a process modification that permits the production of many cast composite material particle/matrix alloy compositions that are difficult to prepare because the matrix alloy does not wet the particles. No new alloying ingredients or atmospheric additions are required, the particles need not be coated, and the temperature is not raised over that normally used. The cost of the production operation remains essentially unchanged from that of conventional procedures. In some instances the quality of the resulting composite materials is surprisingly improved over anything previously known.

In accordance with this feature of the invention and as defined in claim 1, a process for preparing a cast composite material having particles embedded in an aluminum-alloy matrix of a preselected composition that does not readily wet the particles comprises the steps of providing a molten mixture of the particles and a wetting alloy having a composition that readily wets the particles and has no alloying elements present in an amount substantially in excess of the preselected matrix composition; mixing together the molten mixture under conditions such that the wetting alloy is wetted to the particles; adding additional alloying ingredients to the melt to adjust the composition of the matrix to the preselected composition and distributing the additional alloying ingredients throughout the melt; and casting the resulting melt. Preferred embodiments of the claimed process according to claim 1 are given in the dependent claims 2 to 11.

This technique rests upon the realization that some matrix alloy compositions enhance wetting of particular particle types, and other compositions impede wetting. When a difficult-to-wet combination of particle and matrix alloy composition is to be prepared, according to the present invention the matrix alloy is evaluated for the presence of either wettability enhancing elements, combinations, or amounts, or wettability inhibiting elements, combinations, or amounts.

If such enhancing or inhibiting compositions can be identified for a composite system, a wetting alloy composition is designed to take advantage of that situation. The wetting alloy must contain not more than the required amount of each element in the final matrix alloy composition, but can contain less or none. Wetting of the matrix to the particles is then achieved with the wetting alloy. After wetting is accomplished, the composition of the matrix is adjusted with further alloying additions to reach the desired final matrix composition.

It is also provided a cast composite material having a metallic alloy matrix component whose composition is carefully selected to avoid the formation of unwanted and deleterious phases during preparation, remelt, and final casting. The amount of one alloying ingredient is carefully controlled to prevent degradation of properties during remelting, formation of unwanted phases, and good castability. Other conventional alloying ingredients can be varied as necessary to attain other desirable properties of the final product. The particulate need not be altered or specially selected in order to attain good composite remelt properties.

The composite material comprises a mixture of from about 5 to about 35 volume percent of nonmetallic reinforcing particles and from about 95 to about 65 volume percent of a matrix alloy, the matrix alloy being an aluminum-based alloy containing from about 8.5 to about 12.6 weight percent silicon. Other conventional aluminum alloying elements can be added to the matrix alloy as needed, and do not interfere with the beneficial effects of the silicon. Such other alloying elements include, for example, copper, nickel, magnesium, iron and manganese.

The composite material of the invention is particularly useful in remelt applications. It can be remelted to a conventional foundry remelt practice temperature of greater than 700°C, and typically 788°C or more, and held for 24 hours, and then cast with good results. In a preferred embodiment having from about 9.5 to about 11.0 weight percent silicon, the same good casting results are attained with even further improved microstructures in the cast final product.

The present invention provides an important advance in the art of preparation of cast composite materials. Composite-materials can be prepared from materials combinations that are otherwise not commercially feasible, without adding special alloying ingredients or gases that might adversely affect the final product, without specially coating the particles, and without raising the temperature to unacceptably high levels.

The present invention also provides an important advance in the art of cast composite materials, by providing a foundry remelt alloy that can be readily cast by conventional remelt practices. Other features and advantages of the invention will be apparent from the following more detailed description of the preferred embodiment, taken in conjunction with the accompanying drawings, which illustrate, by way of example, the principles of the invention.

### BRIEF DESCRIPTION OF THE DRAWINGS

Figure 1 is a schematic illustration of a fluidity testing apparatus;
Figure 2 is a graph of fluidity test results as a function of silicon content;
Figure 3 is a micrograph of a cast composite material having an aluminum-based matrix containing 7 weight percent silicon;
Figure 4 is a micrograph of a cast composite material having an aluminum-based matrix containing 10 weight percent silicon;
Figure 5 is a micrograph of a cast composite material having aluminum-based matrix containing 10 weight percent silicon and additional alloying elements; and
Figure 6 is a micrograph of another cast composite material having an aluminum-based matrix containing 10 weight percent silicon and additional alloying elements.

### BEST MODES FOR CARRYING OUT THE INVENTION

In accordance with the first embodiment of the invention, a process for preparing a cast composite material having particles embedded in a matrix of a preselected composition that wets the particles only with great difficulty comprises the steps of providing a molten mixture of the particles and a molten Al-wetting alloy having a composition of the preselected matrix composition but with a deficiency in a wettability inhibiting element, the wetting alloy being readily wetted to the particles during mixing; mixing together the molten mixture to wet the wetting alloy to the particles under conditions that the particles are distributed throughout the volume of the melt and the particles and the metallic melt are sheared past each other to promote wetting of the particles by the melt, the mixing to occur while minimizing the introduction of any gas into, and while minimizing the retention of any gas within, the mixture of particles and molten metal, and at a temperature whereat the particles do not substantially chemically degrade in the molten metal in the time required to complete said step of mixing; adding the wettability inhibiting elements to the melt so that the matrix has the preselected composition; and casting the resulting melt at a casting temperature sufficiently high that substantially no solid metal is present.

For the purposes of describing the preferred embodiments of the present invention, cast composite materials can be classified into two groups, those with chemically highly reactive particles and those with chemically nonreactive particles. The principal obstacle with forming cast composite materials containing reactive particles is to prevent particle dissolution and unwanted formation of intermetallic compounds, while achieving wetting. The commercially most important reactive particle is silicon carbide. The principal problem with forming cast composite materials containing nonreactive particles is achieving some degree of reactivity and wetting. The commercially most important nonreactive particle is aluminum oxide. In each case, sufficient fluidity must be exhibited by the melt for casting.

According to one preferred embodiment of the invention for dealing with reactive particles, a process for preparing a cast composite material having particles embedded in an aluminum-alloy matrix having more than about 7 weight percent silicon comprises the steps of providing a molten mixture of the particles, and an aluminum-based wetting alloy having no more than about 7 weight percent silicon; mixing together the molten mixture under conditions such that the aluminum wetting alloy is wetted to the particles; making an addition of silicon and other elements as needed to adjust the silicon content of the melt to its desired final composition which has more than about 7 weight percent silicon, and dissolving and distributing the addition throughout the melt; and casting the resulting melt.

A particularly useful cast composite material has reactive silicon carbide particles embedded in an aluminum-alloy matrix with about 10 weight percent silicon. Castings of this alloy can be made only with great difficulty using the approach of combining all of the ingredients together and mixing. Although the alloy can be mixed, the particulate matter enters the melt slowly, and the melt becomes so viscous that it is difficult to cast.

To prepare such an alloy by the preferred approach, a wetting alloy of aluminum plus about 7 weight percent silicon is prepared and mixed with silicon carbide particles using the approach discussed in US patents 4,759,995 and 4,786,467. Wetting of the wetting alloy to the particles is readily accomplished in about 1 hour of mixing, and the viscosity is acceptable. An addition of the remaining silicon and any other alloying additions required to adjust the matrix to the required alloy content is then made, those additions are dissolved and distributed throughout the volume of the melt, and the melt is cast.

The improvement achieved by the above process is quite surprising. Normally, the fluidity of aluminum-silicon alloys increases with increasing silicon content. Achieving better wetting with a lower silicon content alloy is not expected.

The cast composite material containing silicon preferably comprises a mixture of from about 5 to about 35 volume percent of silicon carbide particles and from about 95 to about 65 volume percent of a cast matrix alloy, the matrix alloy being an aluminum-based alloy containing from about 9.5 to about 11.0 weight percent silicon. Most preferably, the silicon content is about 10 percent by weight of the matrix.

In accordance with a processing aspect of the invention, a method for preparing a cast composite material comprises the steps of preparing molten mixture of from about 5 to about 35 volume percent of free-flowing nonmetallic reinforcing particles and from about 95 to about 65 volume percent of a matrix alloy, the matrix alloy being an aluminum-based alloy containing from about 8.5 to about 12.6 weight percent silicon; mixing the molten mixture to wet the matrix alloy to the particles and to distribute the particles throughout the volume of the melt, the mixing to occur while minimizing the introduction of gas into and retention of gas within the molten mixture; casting the molten mixture; remelting the cast mixture at a temperature that reaches at least about 700°C; and recasting the remelted mixture.

The particles are preferably silicon carbide, because of their light weight and inexpensive commercial availability in suitable forms and sizes. Other nonmetallic reinforcing particles such as other carbides, oxides, nitrides, solicides, and borides, may also be used. The particles must be "free-flowing" in the sense that they are not constrained against movement to reach a uniform distribution throughout the composite material, and are not attached or constrained by a substrate or each other, as is the case for elongated fibers.

The particles constitute from about 5 to about 35 volume percent of the composite material. If less than about 5 volume percent is present, the composite material does not achieve properties superior to those of the conventional, non-composite material. Potentially incurring the problems of a composite material is therefore not justified by superior properties. If more than about 35 volume percent is present, the composite material is so viscous that it cannot be cast. This upper limit to the amount of particulate material can vary somewhat with the shape and type of the particulate material.

The remainder of the composite material, from about 95 to about 65 percent by volume, is the matrix alloy. The matrix alloy is an aluminum-based alloy containing from about 8.5 to about 12.6 weight percent silicon, balance aluminum and other alloying ingredients selected to impart particular mechanical and physical properties to the final solid composite material. Preferably, the silicon content of the matrix is from about 9.5 to about 11.0 weight percent.

The high silicon level has several important functions. The silicon influences the formation of the intermetallic compound aluminum carbide, Al₄C₃, and in particular suppresses its formation. When molten aluminum is contacted to a carbide such as silicon carbide, the formation of aluminum carbide is thermodynamically favoured by a negative free energy of formation. The aluminum carbide is hygroscopic and will absorb moisture. The result is porosity in the final cast product.

The kinetics of aluminum carbide formation have been discovered to be such that melting and mixing of a cast composite material haivng a conventional aluminum-7 (or less) weight percent silicon alloy matrix at a controlled temperature of, for example, about 718°C for a relatively short period of time of about one hour, permits only a small and acceptable amount of the aluminum carbide to form. Thus, an acceptable cast composite material can be prepared by a carefully controlled melting and mixing procedure.

If, however, the cast composite material having such a conventional matrix alloy is thereafter remelted in a foundry practice of 788°C for 24 hours, the aluminum carbide formation continues at an accelerated rate. Aluminum carbide intermetallic compound grows from silicon carbide particles as outwardly projecting needles, which can break off to form particles in the melt.

One potential solution would be to place tight operational controls on foundries. Such controls would not be accepted by some foundries, and in all cases would inhibit the introduction and use of the cast composite materials in applications where they would otherwise be useful.

It has now been discovered that carefully selected larger amounts of silicon in the matrix alloy suppress aluminum carbide formation even during extended holding periods at very high temperatures sufficiently to permit casting of the composite material. The remelted composite materials having the higher silicon content within particular ranges simultaneously achieve exceptional castability and fluidity, without occurrence of primary phases such as pure silicon. Amounts of silicon greater than about 8.5 percent result in significantly reduced aluminum carbide formation and improved remelt fluidity, and amounts of silicon greater than about 9.5 percent eliminate aluminum carbide formation entirely and result in the greatest remelt fluidity for the selected particulate content and remelt temperature and holding conditions.

Castability and fluidity of remelt alloys are of direct interest to foundrymen, because improvements on these characteristics have direct consequences in the ability to cast intricate parts in a reproducible manner. The composite materials of the invention have been comparatively tested to measure their fluidity under typical foundry remelt conditions. Figure 1 illustrates a device 10 for measuring fluidity. Molten composite material 12 is held in a heated crucible 14, with the temperature measured by a thermocouple 16. One end of a hollow pyrex glass tube 18, here about 5 millimetres inside diameter, is inserted vertically into the melt 12. A vacuum of about 63.5 cm of mercury is applied to the other end of the tube 18 by a vacuum pump 20. Molten composite material is drawn up the inside of the tube 18 until the metallic portion of the composite material freezes. The tube 18 is removed from the melt, and the distance of travel of the composite material up the tube prior to freezing is measured.

A number of specimens of composite material were evaluated using the apparatus of Figure 1. Two kilogram heats were prepared with 20 volume percent silicon carbide particles in an aluminum-alloy matrix containing varying amounts of silicon as an alloying ingredient. Melts were prepared with matrix silicon contents of 7, 8, 9, 10, 11, 12, and 13 weight percent silicon. The melts were prepared in a mixer like that disclosed in US Patents 4,759,995 and 4,786,467. The melts were cast into molds and solidified. The castings were remelted in crucibles under air at a temperature of 788°C and held for 24 hours. The temperature of the melt was reduced to 690°C +/6°C, and tested for fluidity using the apparatus of Figure 1.

Figure 2 presents the height rise for the composite materials in inches above the melt level. The greater the height rise, the greater the fluidity. The fluidity increases from a low value at 7 weight percent silicon, to a level at 10 weight percent silicon that remains nearly constant with further increases in silicon content to 13 weight percent. Specimens were cut from the tubes and examined metallographically. The amount of aluminum carbide in the 7 weight percent silicon material was large. A much smaller amount was visible in the sample containing 8 weight percent silicon. There was no aluminum carbide visible in the alloys containing 9 weight percent or more of silicon.

From these data, it was concluded that the minimum silicon content for suppression of aluminum carbide formation, in conditions of extended exposure, together with attainment of acceptable fluidity was about 8.5 percent. This value is marginal, as the aluminum carbide is nearly completely absent, but the fluidity has not reached its greatest value. A preferred minimum silicon content was therefore selected to be about 9.5 weight percent, a level at which no aluminum carbide is present and the fluidity has nearly reached its highest level.

Although the fluidity appears to increase with ever-increasing silicon content within this general range, there is a maximum limit to the silicon content of the matrix alloy. The maximum silicon content of the matrix alloy according to the present invention is about 12.6 weight percent. This is the value of the aluminum-silicon eutectic composition. For greater amounts of silicon, there are two undesirable results. First, the liquidus temperature rises so that the superheat for a selected remelt temperature is reduced. Second, primary silicon particles are precipitated in the matrix upon solidification. The silicon particles reduce the ductility of the matrix. A preferred maximum silicon content is slightly lower, at 11.0 percent.
Metallographic studies reveal that, in the range 11.0-12.6 weight percent silicon, there can be some precipitation of primary silicon in the final structure, regardless of the expected equilibrium phase diagram. Also, there is observed some shrinkage of the matrix alloy during solidification.

The minimum silicon content of the matrix of the present composite material is therefore about 8.5 weight percent, and the preferred minimum is about 9.5 weight percent. The maximum silicon content of the matrix of the present composite material is about 12.6 percent, and the preferred maximum is about 11.0 percent. These values are selected because of, and in conjunction with, the presence of the free-flowing reinforcement particles in the composite material and the potential for chemical interaction between the matrix alloy and the particles as has been discussed herein. The choice of silicon content in non-composite alloys, and alloys that are not to be cast, is therefore not pertinent to the selection of silicon levels for the matrices of cast composite materials.

Most preferably, the silicon content is about 10 weight percent of the matrix, to provide a margin of error between the preferred limits of 9.5 and 11.0 weight percent, and to achieve close to the maximum fluidity possible in this general range.

The silicon in the matrix appears to suppress the formation of aluminum carbide by altering the thermodynamic equilibria of the system. To a good approximation, these equilibria are not affected by the presence of metallic alloying elements commonly provided in aluminum alloys to achieve specific properties such as strength, toughness, corrosion resistance, and the like in the final cast product. Thus, superior casting performance can be achieved by maintaining the proper silicon content, and other alloying elements can be added to achieve specific properties in the final product. Such alloying elements include, for example, copper, nickel, magnesium, iron, and manganese.

The following examples are presented in addition to those discussed previously to illustrate aspects of the invention, but are not intended to limit the invention in any aspect.

### Example 1

To prepare a cast composite material of 20 volume percent of silicon carbide particles in a matrix alloy of 10 weight percent silicon, 1 weight percent magnesium, balance aluminum, a wetting alloy of 7 weight percent silicon, 1 weight percent magnesium, balance aluminum was prepared. The appropriate amounts of silicon carbide and the wetting alloy were mixed according to the procedures disclosed in US Patent 4,759,995 and 4,786,467. More specifically, the wetting alloy was melted at 671°C, and the appropriate amount of silicon carbide particles was added to the surface of the melt under vacuum over a period of 35 minutes, while the melt was mixed with an impeller. After all the silicon carbide was added, mixing was continued for another 25 minutes under vacuum. This procedure produced full wetting of the aluminum-7 weight percent silicon, 1 weight percent magnesium alloy to the particles. The mixing was stopped, the chamber vented to air, and a sufficient amount of silicon was added to adjust the matrix composition to 10 weight percent silicon and 1 weight percent magnesium. The chamber was sealed and a vacuum drawn, and mixing was continued for another 15 minutes to dissolve the alloying additions and distribute them throughout the melt. The composite material was cast into pigs. The pigs were provided to a foundry for remelt, and the remelted composite material was observed to have excellent fluidity for casting into narrow mold passages.

### Example 2

Example 1 was repeated, except that stepped alloying was not used. That is, the conventional practice was followed wherein the final matrix alloy of 10 weight percent silicon, 1 weight percent magnesium, balance aluminum was prepared. Silicon carbide particulate in the appropriate amount was added to the melt, and the melt and particles mixed together for the same amount of time as in Example 1. The resulting melt was very viscous and could not be cast into small-diameter passages in molds.

### Example 3

Example 1 is repeated, except that the composite was made to contain 10 volume percent of silicon carbide particles. The final melt was fluid and could be cast into molds with both large and small passageways.

### Example 4

Example 2 was repeated, Except that the composite was made to contain 10 volume percent of silicon carbide particles.

### Example 5

The mechanical properties of cast specimens of the stepped-alloy addition cast composite material of Example 3 and the conventionally prepared cast composite material of Example 4 were tested. The following table reports the results in ksi, thousands of pounds per square inch.

**Table 1**

| | Yield Strength | | Tensile Strength | |
|---|---|---|---|---|
| Process | (ksi) | (Mpa) | (ksi) | (Mpa) |
| Prior | 42 | 290 | 47 | 324 |
| Stepped | 49 | 338 | 56 | 386 |

The composite materials produced with the stepped addition of alloying ingredients exhibit significantly improved post-casting properties as compared with those produced by the conventional approach.

The second class of particles is nonreactive particles such as aluminum oxide particles. According to another preferred embodiment of the invention for dealing with nonreactive particles, a process for preparing a cast composite material having particles embedded in an aluminum-alloy matrix comprises the steps of providing a molten mixture of the particles, and an aluminum-based wetting alloy having about 1 weight percent silicon and about 0.6 weight percent magnesium; mixing together the molten mixture under conditions such that aluminum wetting alloy is wetted to the particles; making an addition of elements as needed to adjust the alloy content of the melt to its desired final composition, and dissolving and distributing the addition throughout the melt; and casting the resulting melt.

To prepare a cast composite material containing nonreactive particles, the particles are first mixed with a wetting alloy which is known to wet the particles and also has sufficient fluidity for mixing. For example, it is known that aluminum alloys containing about 1 weight percent silicon and 0.6 weight percent magnesium readily wet aluminum oxide particles during mixing. Many aluminum matrix alloys of interest contain at least 1 weight percent silicon and at least 0.6 weight percent magnesium, so initial wetting can be accomplished with an aluminum alloy of that composition. After wetting, the composition of the matrix is adjusted with further additions of alloying elements. The initial wetting is accomplished using the wetting alloy and the procedure of US Patents 4,759,995 and 4,786,467.

The following example is intended to illustrate aspects of the invention as related to wetting of nonreactive particles.

### Example 6

This example illustrates aspects of the invention as related to wetting of nonreactive particles.

A cast composite material was prepared of 10 volume percent aluminum oxide particles in an aluminum alloy containing 10 weight percent silicon, 0.6 weight percent magnesium, 0.7 weight percent iron, and 0.4 weight percent manganese. This cast composite material is exceedingly difficult to prepare by conventional methods, because the particles wet only slowly. The molten composite material is so viscous that it is nearly impossible to cast into a mold. To prepare the cast composite material using the approach of the invention, a matrix alloy of 1 weight percent silicon, 0.6 weight percent magnesium, 0.7 weight percent iron, and 0.4 weight percent manganese, balance aluminum, was melted in a crucible at 674°C under vacuum, and the appropriate amount of aluminum oxide particles added over a period of 20 minutes. The aluminum-based matrix alloy contains 1 weight percent silicon and 0.6 weight percent magnesium, a composition known to achieve wetting to aluminum oxide particles. After all of the particulate matter was added, the melt was mixed under vacuum for another 20 minutes, following the approach of US Patents 4,759,995 and 4,786,467. This combination of matrix alloy composition and mixing conditions produced good wetting of the matrix alloy to the particles. Mixing was stopped, the chamber was vented to air, and sufficient silicon added to adjust the matrix content to 10 weight percent silicon (with the amounts of the other alloying additions essentially unchanged). The vacuum was reapplied, and mixing continued for another 15 minutes. The composite was then cast into foundry pigs. The cast composite material exhibited excellent fluidity, and was suitable for preparation of castings having narrow passageways.

### Example 7

A cast composite material was prepared from 20 volume percent silicon carbide particles and 80 volume percent of an alloy meeting a specification of 7 weight percent silicon, 0.3-0.45 weight percent magnesium, balance aluminum. This matrix alloy is not within the scope of the invention, and is presented for comparative purposes. The cast composite material was prepared by the procedures discussed previously. The cast composite material was remelted at a temperature of over 760°C. A sample was taken of the remelted composite material, and its microstructure is illustrated in Figure 3. Aluminum carbide intermetallic compound is found extensively throughout the microstructure as a dark-appearing phase. In Figure 3, circles have been drawn around some of the aluminum carbide particles and regions for illustrative purposes.

### Example 8

Example 7 was repeated, except using a matrix alloy that meets a specification of 10 weight percent silicon, 0.8-1.0 weight percent magnesium, balance aluminum. Except for the higher silicon content within the preferred range of the invention and a minor difference in magnesium content, this matrix alloy has the same composition as that of Example 7. The microstructure of this alloy is shown in Figure 4. There is no aluminum carbide visible in the microstructure.

### Example 9

Example 7 was repeated, except using a matrix alloy that meets a specification of 10 weight percent silicon, 0.6-1.0 weight percent iron, 3.0-3.5 weight percent copper, 0.2-0.6 weight percent manganese, 0.3-0.6 weight percent magnesium, 1.0-1.5 weight percent nickel, balance aluminum. This matrix alloy is within the scope of the invention, having 10 weight percent silicon. It is a more complex alloy in that it also contains iron, copper, manganese, and nickel. This cast composite material is suitable as a die casting alloy. Figure 5 illustrates the microstructure of this cast and then remelted alloy. There is no aluminum carbide visible in the microstructure.

### Example 10

Example 7 was repeated, except using a matrix alloy that meets a specification of 10 weight percent silicon, 2.8-3.2 weight percent copper, 0.8-1.2 weight percent magnesium, 1.0-1.5 weight percent nickel, balance aluminum. This matrix alloy contains copper and nickel in addition to the silicon within the range of the invention and magnesium. This composite material is suitable as a high temperature sans and permanent mold casting alloy. Figure 6 illustrates the microstructure of this cast and remelted alloy. There is no aluminum carbide visible in the microstructure.

Example 8 demonstrates that the addition of silicon to within the range of the invention suppresses aluminum carbide formation, as compared with the alloy of Example 7. Examples 9 and 10 demonstrate that additions of other alloying elements do not interfere with the suppression of aluminum carbide formation by the high silicon content. The results of Figure 2 demonstrate that the 10 weight percent silicon alloy has excellent fluidity and it was observed to have good castability.

In the preceeding disclosure and Examples 1-6, procedures for achieving acceptable wetted cast composite materials of both reactive and nonreactive particles have been demonstrated. In each case, composite materials that are difficult to make by the conventional approach are prepared using the conventional mixing procedure and a matrix alloy that is known to be operable to first achieve wetting of the matrix alloy to the particles, and thereafter adjusting the composition of the matrix to the preselected alloying level. In each case, no coatings on the particles, special alloying elements, special atmospheric additions, or overly elevated temperatures are required. The only changes to the processing procedures are to add some alloying elements after wetting is complete, and to extend the mixing for a short time to incorporate these later additions into the melt.

The composite material of the invention provides an important commercial advance in the art of cast composite materials. The material can be mixed and cast by a primary composite material supplier, and shipped as a cast ingot to a foundry for remelting and casting into precise shapes as required. The composition of the matrix alloy is selected so that the remelting practice at the foundry may be similar to conventional remelt practices, which would not be possible for a cast composite material of conventional alloying content. Excellent fluidity is retained by the molten composite material even when it is held in a remelt crucible for extended periods of time and at temperatures previously thought to be unacceptably high because they produce undesirable reaction products.

## Claims

1. A process for preparing a cast composite material having particles embedded in a metal alloy matrix of a preselected composition that wets the particles only with great difficulty, comprising the steps of:
combining free-flowing non-metallic reinforcing particles and a molten aluminum wetting alloy having a composition of the preselected matrix composition but with a deficiency in wettability inhibiting elements, the wetting alloy being capable of being wetted to the particles by mixing;
mixing together the combined free-flowing particles and molten aluminum wetting alloy to wet the wetting alloy to the particles under conditions that the particles are distributed throughout the volume of the melt and the particles and the aluminum melt are sheared past each other to promote wetting of the particles by the melt, the mixing being carried out while minimizing the introduction of any gas into, and while minimizing the retention of any gas within, the mixture of particles and molten aluminum, and at a temperature at which the particles do not substantially chemically degrade in the molten aluminum in the time required to complete said step of mixing;
thereafter adding the wettability inhibiting elements to the mixture of particles and molten aluminum wetting alloy so that the matrix has the preselected composition; and
casting the resulting molten mixture at a casting temperature sufficiently high that substantially no solid metal is present.

2. The process as claimed in claim 1, characterized in that the non-metallic reinforcing material is a refractory ceramic selected from the group consisting of a metal oxide, metal nitride, metal carbide, metal silicide, and a glass.

3. The process of claim 1 or 2, characterized in that the wetting aluminum alloy has no more than about 7 weight percent silicon.

4. The process as claimed in any one of claims 1-3, characterized in that the wetting alloy has about 1.0 weight percent silicon and about 0.8 weight percent magnesium.

5. The process as claimed in claim 3, characterized in that silicon is added to the mixture as the wettability inhibiting element to produce a final composite material containing more than about 7 weight percent silicon.

6. The process as claimed in any one of claims 1-5, characterized in that the final composite material contains about 5 to about 35 volume percent of said particles.

7. The process as claimed in any one of claims 1-6, characterized in that the final composite material contains about 8.5 to about 12.6 weight percent silicon.

8. The process as claimed in any one of claims 1-6, characterized in that the final composite material contains about 9.5 to about 11.0 weight percent silicon.

9. The process as claimed in any one of claims 1-8, characterized in that the particles are silicon carbide.

10. The process as claimed in any one of claims 1-8, characterized in that the particles are aluminum oxide.

11. The process as claimed in any one of claims 1-8, characterized in that the cast composite material obtained is remelted and recast.

## Patentansprüche

1. Verfahren zur Herstellung eines gegossenen Verbundstoffs mit Teilchen, die in einer diese nur sehr schwer benetzenden Metallegierungsmatrix einer vorgewählten zusammensetzung eingebettet sind, umfassend folgende Stufen:
Kombinieren fließfähiger nichtmetallischer Verstärkungsteilchen und einer schmelzflüssigen Aluminiumbenetzungslegierung mit der Zusammensetzung der vorgewählten Matrixzusanmensetzung, aber mit einem Mangel an die Benetzbarkeit hemmenden Elementen, wobei die Benetzüngslegierung die Teilchen durch Vermischen benetzen kann;
Vermischen der mit der schmelzflüssigen Aluminiumbenetzungslegierung kombinierten fließfähigen Teilchen, um diese mit der Benetzungslegierung unter solchen Bedingungen zu benetzen, daß die Teilchen über das Gesamtvoluwen der Schmelze verteilt sind, und die Teilchen und die Aluminiumschmelze zur Förderung der Benetzung der Teilchen mit der Schmelze aneinander vorbeischeren, wobei das Vermischen so erfolgt, daß die Einführung jeglichen Gases in das Gemisch aus Teilchen und schmelzflüssigem Aluminium sowie die Rückhaltung jeglichen Gases darin auf ein Mindestmaß beschränkt sind, bei einer Temperatur, bei der die Teilchen innerhalb der zur Vollendung besagter Mischstufe erforderlichen Zeit in dem schmelzflüssigen Aluminium chemisch nicht wesentlich abgebaut werden;
danach Zugabe der die Benetzbarkeit hemmenden Elemente zu dem Gemisch aus Teilchen und schmelzflüssiger Aluminiumbenetzungslegierung, so daß die Matrix die vorgewählte zusammensetzung besitzt; und
Gießen des so erhaltenen schmelzflüssigen Gemischs bei einer genügend hohen Gießtemperatur, so daß im wesentlichen kein festes Metall vorliegt.

2. Verfahren nach Anspruch 1, dadurch gekennzeichnet, daß das nichtmetallische Verstärkungsmaterial ein aus der Metalloxid, Metallnitrid, Metallcarbid, Metallsilicid und Glas umfassenden Gruppe ausgewählter feuerfester keramischer Stoff ist.

3. Verfahren nach Anspruch 1 oder 2, dadurch gekennzeichnet, daß die Aluminiumbenetzungslegierung nicht mehr als etwa 7 Gew.-% Silicium enthält.

4. Verfahren nach einem der Ansprüche 1-3, dadurch gekennzeichnet, daß die Benetzungslegierung etwa 1,0 Gew.-% Silicium und etwa 0,8 Gew.-% Magnesium enthält.

5. Verfahren nach Anspruch 3, dadurch gekennzeichnet, daß man dem Gemisch Silicium als die Benetzbarkeit hemmendes Element zusetzt, um einen fertigen Verbundstoff zu erzeugen, der nicht mehr als etwa 7 Gew.-% Silicium enthält.

6. Verfahren nach einem der Ansprüche 1-5, dadurch gekennzeichnet, daß der fertige Verbundstoff etwa 5 bis etwa 35 Vol.-% besagter Teilchen enthält.

7. Verfahren nach einem der Ansprüche 1-6, dadurch gekennzeichnet, daß der fertige Verbundstoff etwa 8,5 bis etwa 12,6 Gew.-% Silicium enthält.

8. Verfahren nach einem der Ansprüche 1-6, dadurch gekennzeichnet, daß der fertige Verbundstoff etwa 9,5 bis etwa 11,0 Gew.-% Silicium enthält.

9. Verfahren nach einem der Ansprüche 1-8, dadurch gekennzeichnet, daß die Teilchen aus Siliciumcarbid bestehen.

10. Verfahren nach einem der Ansprüche 1-8, dadurch gekennzeichnet, daß die Teilchen aus Aluminiumoxid bestehen.

11. Verfahren nach einem der Ansprüche 1-8, dadurch gekennzeichnet, daß der erhaltene gegossene Verbundstoff nochmals geschmolzen und gegossen wird.

## Revendications

1. Un procédé pour préparer un matériau composite coulé ayant des particules noyées dans une matrice d'alliage métallique d'une composition présélectionnée qui ne mouille les particules seulement qu'avec grande difficulté, comprenant les étapes consistant à :
combiner des particules de renforcement non-métalliques s'écoulant librement avec un alliage de mouillage d'aluminium en fusion ayant une composition de la composition de matrice présélectionnée mais avec une déficience en éléments inhibiteurs de mouillabilité, l'alliage de mouillage étant capable de mouiller les particules par mélange;
mélanger ensemble les particules s'écoulant librement et l'alliage de mouillage d'aluminium en fusion combinés pour mouiller les particules avec l'alliage de mouillage sous les conditions que les particules sont réparties à travers tout le volume du bain et que les particules et le bain d'aluminium soient cisaillés l'un dans l'autre pour provoquer le mouillage des particules par le bain, le mélange étant effectué tout en minimisant à la fois l'introduction d'un gaz quelconque et la rétention d'un gaz quelconque à l'intérieur du mélange de particules et d'aluminium en fusion, et à une température à laquelle les particules ne subissent substantiellement pas de dégradations chimiques dans l'aluminium en fusion pendant le temps nécessaire à l'accomplissement de ladite étape de mélange;
ajouter après cela les éléments inhibiteurs de mouillabilité au mélange de particules et d'alliage de mouillage d'aluminium en fusion de telle façon que la matrice ait la composition présélectionnée; et
couler le mélange en fusion résultant à une température de coulée suffisamment élevée pour que substantiellement aucun métal solide ne soit présent.

2. Le procédé suivant la revendication 1, caractérisé en ce que le matériau de renforcement non-métallique est une céramique réfractaire choisie dans le groupe consistant en un oxyde de métal, un nitrure de métal, un carbure de métal, un siliciure de métal et un verre.

3. Le procédé suivant la revendication 1 ou 2, caractérisé en ce que l'alliage d'aluminium de mouillage n'a pas plus de 7 % en poids de silicium.

4. Le procédé suivant l'une quelconque des revendications 1 à 3, caractérisé en ce que l'alliage de mouillage a environ 1,0 % en poids de silicium et environ 0,8 % en poids de magnésium.

5. Le procédé suivant la revendication 3, caractérisé en ce que le silicium est ajouté au mélange comme élément inhibiteur de mouillabilité pour produire un matériau composite final contenant plus qu'environ 7 % en poids de silicium.

6. Le procédé suivant l'une quelconque des revendications 1 à 5, caractérisé en ce que le matériau composite final contient en volume d'environ 5 % à environ 35 % desdites particules.

7. Le procédé suivant l'une quelconque des revendications 1 à 6, caractérisé en ce que le matériau composite final contient en poids d'environ 8,5 % à environ 12,6 % de silicium.

8. Le procédé suivant l'une quelconque des revendications 1 à 6, caractérisé en ce que le matériau composite final contient en poids d'environ 9,5 % à environ 11,0 % de silicium.

9. Le procédé suivant l'une quelconque des revendications 1 à 8, caractérisé en ce que les particules sont du carbure de silicium.

10. Le procédé suivant l'une quelconque des revendications 1 à 8, caractérisé en ce que les particules sont de l'oxyde d'aluminium.

11. Le procédé suivant l'une quelconque des revendications 1 à 8, caractérisé en ce que le matériau composite coulé obtenu est refondu et recoulé.
